

Dec. 16, 1941.

A. M. TALBOT

2,266,481

AGE HARDENABLE, LOW EXPANSION, NICKEL-IRON-TITANIUM ALLOY

Filed Oct. 27, 1939

2 Sheets-Sheet 1

Fig. 1.



Fig. 2.



INVENTOR

ALBERT M. TALBOT

BY

*A. M. Talbot*  
ATTORNEY

Dec. 16, 1941.

A. M. TALBOT

2,266,481

AGE HARDENABLE, LOW EXPANSION, NICKEL-IRON-TITANIUM ALLOY

Filed Oct. 27, 1939

2 Sheets-Sheet 2

Fig. 3.



Fig. 4.



Fig. 5.



## UNITED STATES PATENT OFFICE

2,266,481

AGE HARDENABLE, LOW EXPANSION,  
NICKEL-IRON-TITANIUM ALLOY

Albert M. Talbot, Fairhaven, N. J., assignor to  
The International Nickel Company, Inc., New  
York, N. Y., a corporation of Delaware

Application October 27, 1939, Serial No. 301,580

3 Claims. (Cl. 148—31)

The present invention relates to improved low expansion iron-nickel alloys and articles of manufacture made therefrom, and more particularly to improved age-hardenable iron-nickel alloys with predictable low expansion characteristics containing correlated and balanced amounts of nickel and hardening agent, and to age hardened articles of manufacture made therefrom.

The anomalous expansion characteristics of iron-nickel alloys containing from about 30% to 50% nickel are well known. Ferro-nickel alloys with about 36% nickel have very low coefficients of expansion, which approach zero for a temperature range up to about 300° or 400° F. As the nickel content is decreased from 36%, the coefficient of expansion rises rapidly above that obtained with 36% nickel and the temperature range of low expansivity is lowered. On the other hand, as the nickel content is increased above 36%, the coefficient of expansion rises more slowly and at the same time, the temperature range over which the alloy will display low expansion characteristics is raised. It is possible by regulating the nickel content between about 36 and 50% to obtain any desired coefficient of expansion between  $0.5 \times 10^{-6}$  per °F. and  $5.5 \times 10^{-6}$  per °F. The various properties of these iron-nickel alloys are well known and amply described in the literature, e. g., Scott's article in Transactions of the American Society for Steel Treating, vol. 13, 1928, p. 829. The low expansion iron-nickel alloys are known under various trademarks. The 36% nickel alloy is known as Invar, while the 46% nickel alloy has the same coefficient as platinum and is known as Platinite. These austenitic alloys can be hardened by cold work. When the alloys were hardened only by cold work, many potential applications were limited by the fact that the ordinary alloys did not possess the required high strength, hardness, elastic properties, wear resistances, etc. It was known that appropriate amounts of titanium will confer age hardenability upon a broad range of austenitic nickel-iron and iron-nickel alloys. When titanium was incorporated in the 36% nickel alloy to impart age hardenability thereto, certain shortcomings were encountered with regard to the expansion properties.

Although many attempts were made to remedy the aforementioned shortcomings, none, as far as I am aware, was entirely successful, produced satisfactory results and could be carried into practical and economic industrial scale operation.

I have discovered that in spite of the presence of titanium it is possible, by critically adjusting the nickel and titanium contents in iron-nickel alloys to provide predetermined expansivity characteristics and to provide low expansivity coupled with high mechanical properties, including hard-

ness, which make the new alloys applicable in many situations where the straight iron-nickel alloys were entirely unsuitable due to their low hardness and particularly their low yield point.

5 It is an object of the present invention to provide improved age hardenable iron-nickel alloys with predetermined low expansion characteristics which contain controlled and adjusted proportions of nickel, carbon and titanium and in which the nickel is balanced against the titanium and the carbon.

It is another object of the present invention to provide age hardenable low expansion iron-nickel alloys containing titanium and characterized by improved mechanical properties, including high tensile strength and high hardnesses, while still being able to control the expansion characteristics by proper control of the chemical composition.

10 It is a further object of the present invention to provide age hardened articles of manufacture made of low expansion iron-nickel-titanium alloys in which the nickel is adjusted in special proportions to compensate for the modification in expansion properties caused by the introduction of titanium into the alloy.

The invention contemplates a method of producing age hardenable iron-nickel alloys containing controlled amounts of titanium, and articles of manufacture made therefrom, possessing predetermined expansion properties combined with high mechanical properties in the age hardened condition, said process involving an adjustment, in special proportions, of the nickel content to compensate for the modification in expansion properties caused by titanium.

Other objects and advantages of the present invention will become apparent to those skilled in the art from the following description taken in conjunction with the accompanying drawings in which:

Fig. 1 is a graph illustrating the effect of non-carbidic titanium upon the hardness of iron-nickel alloys;

45 Fig. 2 is a graph depicting a typical expansion curve;

Fig. 3 is a graph depicting the influence of effective nickel upon the minimum coefficient of expansion of iron-nickel titanium alloys at different representative levels of non-carbidic titanium;

50 Fig. 4 is a graph showing the relation between inflection temperature and effective nickel content in iron-nickel-titanium alloys; and

55 Fig. 5 is a graph showing the solution temperatures and aging temperatures preferably employed in age hardening iron-nickel alloys containing various amounts of non-carbidic titanium.

Table I

|   | Element                    | Percentage   |
|---|----------------------------|--------------|
| 5 | Effective nickel.....      | percent..... |
|   | Total nickel.....          | do.....      |
|   | Non-carbidic titanium..... | do.....      |
|   | Total titanium.....        | do.....      |
|   | Carbon.....                | do.....      |
|   | Iron.....                  | do.....      |

- 10 As pointed out hereinbefore, carbon need not be, but usually is, present due to commercial production methods. It is to be understood that carbon may be completely absent or may be present only in traces or small amounts of the order of 0.001%. In addition to the elements nickel, iron and titanium, and usually carbon, the alloys may also contain small amounts of minor elements and impurities, and when I say in the specification and claims that the "balance is iron," "balance is substantially all iron," etc., I include within the expression minor constituents and impurities, such as cobalt, manganese, silicon, aluminum, sulfur, phosphorus, and other elements commonly present in such materials in commercial practice. Cobalt in appropriate amounts may be beneficial. It is well known that amounts of the order of 5% cobalt are beneficial in ordinary iron-nickel alloys of the Invar type. The alloys may also contain from traces, say 0.001%, up to possibly 1.5% manganese, up to about 1.5% silicon, up to about 1.0% aluminum, etc. From about 0.2% to 0.5% manganese is usually present for forgeability, although about 0.05% calcium may be a desirable alternative addition. Aluminum and silicon are commonly present in commercial ferro-titanium and are often introduced into the alloy along with the titanium. Although silicon contents up to about 0.9% have been used, the silicon content is preferably held to less than about 0.3%, e. g., 0.1 to 0.2%, and the aluminum content does not usually exceed about 0.5%, e. g., 0.3%.
- 15
- 20
- 25
- 30
- 35
- 40

45 More specifically when the lowest expansion properties are desired it is preferred to regulate the nickel, carbon, titanium and iron content in amounts to give the compositions set forth in Table II in accordance with the balanced proportions set forth by the formula given hereinbefore.

Table II

|    | Element                    | Percentage   |
|----|----------------------------|--------------|
| 55 | Effective nickel.....      | percent..... |
|    | Total nickel.....          | do.....      |
|    | Non-carbidic titanium..... | do.....      |
|    | Total titanium.....        | do.....      |
|    | Carbon.....                | do.....      |
|    | Iron.....                  | do.....      |

- 60 After an age hardening treatment the alloys of the present invention possess markedly increased mechanical properties and then exhibit the desired low expansion properties. Thus, Brinell hardnesses as high as 400 are developed after age hardening heat treatment as compared to Brinell hardnesses of about 130 for ordinary, titanium-free, iron-nickel alloys containing about 36% nickel. The maximum physical properties, particularly the proportional limit, obtainable in a fully aged alloy depends upon the amount of non-carbidic titanium present in the alloy. In general, the mechanical properties of aged material increase with the non-carbidic titanium. Fig. 1
- 65
- 70
- 75

$$\text{Effective Ni} = \text{Total Ni} - K(\text{Non-carbidic Ti})$$

In this equation, K is a constant with a value of about 2.4; and for practical purposes, Non-carbidic Ti is equal to  $Ti - 4 \times C$ ; and Ni, Ti and C are nickel, titanium and carbon, respectively, in weight percentage.

The desired Brinell hardness and related mechanical properties determines the titanium content. The desired minimum expansion characteristics determine the effective nickel content which is related to the total nickel content as expressed by the following formula:

$$\text{Total Ni} = \text{Effective Ni} + K(Ti - 4 \times C)$$

In carrying the invention into practice, the compositions of the alloys fall within the approximate ranges given in Table I in balanced proportions as expressed by the formula set forth hereinbefore.

the hardness of alloys produced in accordance with the present invention. Other mechanical properties may be correlated to the Brinell hardness as is well known to those skilled in the art. The hardness reaches a maximum at about 4% non-carbidic titanium but for practical purposes the maximum is reached at about 3.25% non-carbidic titanium since further increases in non-carbidic titanium produce only slightly higher hardnesses and increase the cost and difficulty of manufacture. Increasing the non-carbidic titanium content lowers the inflection temperature. A high inflection temperature is desirable because this means that the minimum expansion region extends to a higher temperature. Fig. 2 is a graph of a typical expansion curve showing the inflection temperature and the range of minimum expansivity. An increase in the non-carbidic titanium also raises the general level of expansivity as shown in Fig. 3, and the over-all expansion through a range of temperatures, and raises the total nickel content required to secure the lowest expansivity. In Fig. 3 the influence of effective nickel content on the minimum coefficient of expansion at two non-carbidic titanium levels is shown. It will be apparent that a balance must be made between the desired hardness or other mechanical property and the desired low expansion properties where, for instance, expansivities below  $2 \times 10^{-6}$  per °F. are required, and that only the amount of non-carbidic titanium necessary to give the desired hardness or other mechanical property should be used. The most favorable balance between properties is had by limiting the non-carbidic titanium content to the lowest amount sufficient to give adequately high mechanical properties. Thus, where it is desired that the alloy have a very high hardness, e. g., 365 Brinell hardness, in combination with the lowest possible minimum coefficient of expansion at that level of hardness, a non-carbidic titanium content of about 2.6%, with an effective nickel content of about 34.5% to 36.5%, is satisfactory. Where a hardness of about 325 Brinell combined with the lowest possible minimum coefficient of expansion is desired a non-carbidic titanium content of about 2.1%, in combination with an effective nickel content of about 34.5% to 36.5%, is satisfactory. In plotting the minimum coefficient of expansion against effective nickel content it is observed from Fig. 3 that the curve becomes comparatively flat in the vicinity of the lowest minimum coefficient of expansion and that a range of effective nickel contents is available which yield substantially similar minimum expansion properties, however, it is preferred to use the higher effective nickel contents in this range since the alloys of higher effective nickel content have higher inflection temperatures. It has been found that the inflection temperature bears no obvious relation to the total nickel content within the ranges contemplated but is simply related to the effective nickel content. This relationship between effective nickel and inflection temperature is shown graphically in Fig. 4. Aluminum has no substantial effect upon the minimum coefficient of expansion but lowers the inflection temperature. Silicon causes an increase in the minimum coefficient of expansion in addition to lowering the inflection temperature. Accordingly, where silicon and/or aluminum must be present, aluminum should be used in preference to silicon and the silicon content held at a low value, e. g., 0.1% to 0.2%. Manganese increases the mini-

mum coefficient of expansion and preferably only that amount required to insure forgeability should be present in the alloy, e. g., 0.3% to 0.5% manganese.

5 The alloys of the present invention possess low or minimum expansion properties and characteristics after age hardening heat treatment. This heat treatment comprises a high temperature solution treatment followed by rapid cooling, e. g., quenching, and then an aging treatment at lower temperatures to effect precipitation of the hardening constituent in a finely divided state followed by cooling, preferably rapid cooling, to atmospheric temperatures. The solution treatment is usually carried out at temperatures within the range of 1650° F. to 1825° F., the lower temperatures being preferably employed for alloys with low "non-carbidic titanium" contents. Lower temperatures may be used, especially with low 10 titanium contents, but more time is required to soften the alloys. The solution temperatures preferably employed are shown in Fig. 5 and lie in a band extending from about 1650° F. to 1725° F. for 1% non-carbidic titanium to about 1750° F. to 1825° F. for 4.25% non-carbidic titanium. 15 A solution heat treatment of about 2 to 3 hours at these temperatures is usually satisfactory, although still longer times are desirable for castings and temperatures of the order of 2000° to 20 titanium contents, but more time is required to 25 soften the alloys. The solution temperatures preferably employed are shown in Fig. 5 and lie in a band extending from about 1650° F. to 1725° F. for 1% non-carbidic titanium to about 1750° F. to 1825° F. for 4.25% non-carbidic titanium. 20 A solution heat treatment of about 2 to 3 hours at these temperatures is usually satisfactory, although still longer times are desirable for castings and temperatures of the order of 2000° to 30 2100° F. may be used. After solution heat treatment the alloys are rapidly cooled. Oil quenching is satisfactory for most section sizes to insure full softening and, of course, a water quench may be used. In general any cooling from solution 35 temperatures which is sufficiently rapid to produce a softened alloy, i. e., an alloy having a hardness not exceeding about 150 to 160 Brinell will be satisfactory. Slow cooling from the solution temperatures results in full hardening, but where lowest expansivity is required this is not a desirable method of obtaining hardening due to the undesirable effects of this method on the 40 expansion characteristics. It has been found that a rapid cooling rate is necessary to obtain the lowest expansion characteristics. The aging treatment is carried out within the somewhat narrow and critical temperature range of 1100° F. to 1325° F. for from about 1 to about 24 hours. 45 The aging temperature preferably increases with the amount of the non-carbidic titanium. The preferred aging temperatures are shown in Fig. 5 and lie in a band extending from about 1100° F. to 1150° F. at 1% non-carbidic titanium to about 50 1250° F. to 1325° F. at 4.25% non-carbidic titanium. The alloys are preferably aged for about 8 to 12 hours although by far the majority of the hardening occurs within the first hour. Low titanium-containing alloys, e. g., about 1% non-carbidic titanium, require longer aging periods 55 up to 24 hours. In general, aging is more rapid as the "non-carbidic titanium" increases. Typical examples of satisfactory aging temperatures for various non-carbidic titanium contents in alloys of the present invention are given in Table III.

Table III

| Percent non-carbidic titanium | Aging temperature<br>° F. |
|-------------------------------|---------------------------|
| 1.51                          | 1,150                     |
| 2.12                          | 1,200                     |
| 2.96                          | 1,250                     |
| 4.19                          | 1,300                     |

Aging for 2 or 3 hours at each of a plurality of successively lower temperatures produces substantially similar hardening to aging 8 to 12 hours at a single proper temperature. After the aging treatment, the alloys may be cooled in any manner but it is preferred to rapidly cool, e. g., water quench, since this produces lower coefficients of expansion than are observed after slow cooling. Satisfactory solution temperatures and aging temperatures for wrought alloys containing various percentages of "non-carbidic titanium" are shown graphically in Fig. 5. A satisfactory heat treatment for a wrought iron-nickel alloy containing about 2.75% noncarbidic titanium (2.81% total titanium) in accordance with the present invention comprises heating for about 2 hours at about 1700° F. followed by oil quenching and aging at about 1250° F. for about 9 hours.

All the mechanical properties do not reach their maximum values after the same aging time. The proportional limit reaches its maximum values early during the aging period and then decreases slightly upon further aging whereas the tensile strength and hardness reach a maximum value at about the normal aging time and the yield point continues to rise slightly when aged beyond normal times. For example, the proportional limit of an alloy containing 2.1% non-carbidic titanium was raised from about 22,000 pounds per square inch to a maximum of about 76,000 pounds per square inch after one hour of aging whereas the tensile strength was raised from about 80,000 pounds per square inch to about 142,000 pounds per square inch in about one hour of aging and to a maximum of about 160,000 pounds per square inch after about nine hours of aging. The yield point of the alloy was raised from about 42,000 pounds per square inch to about 98,000 pounds per square inch in about one hour, to about 114,000 pounds per square inch in about nine hours and to about 118,000 pounds per square inch in eighteen hours.

It has been found that the effect of cold work is decidedly beneficial upon the properties of the alloys. Cold work has the effect of reducing the minimum coefficient of expansion and has greater effect if applied before aging than after aging. Cold working before aging also raises the final hardness as much as 40 to 45 Brinell hardness numbers with 20% to 40% or more of cold reduction. This treatment gives the maximum hardness attainable in a particular alloy. Cold working after aging is less effective and raises the hardness up to about 20 Brinell hardness with 20% or more cold reduction. It is preferred to obtain a desired hardness by cold working and aging an alloy rather than by increasing the "non-carbidic titanium" content and then aging without cold working. In this

manner the best possible expansion properties are obtained in combination with the desired high mechanical properties. It appears that any treatment that produces internal stresses is beneficial in reducing the coefficient of expansion. The maximum aging response in cold worked material is obtained by aging at slightly lower temperatures, e. g., 50° F. lower, than at the regular aging temperatures but the latter temperatures may be used to give very satisfactory results and substantially the same results may be obtained in slightly less time. The minimum coefficient of expansion of aged and quenched material produced in accordance with the present invention is not materially increased by heating for a short time up to temperatures of about 600° F. or for a long time at temperatures up to 350° F. Thus, heating aged material of the present invention for ten days at 350° F. resulted only in a very slight increase in the minimum coefficient of expansion, i. e., from  $1.9 \times 10^{-6}$  per °F. to  $2.1 \times 10^{-6}$  per °F.

Materials having the compositions contemplated by the present invention may be worked in the usual manner into products possessing high mechanical properties combined with low expansion characteristics. Forging operations are preferably carried out at temperatures of about 1800° F. to about 2300° F. followed by quenching or rapid cooling where softened material is desired. Representative approximate values for the properties obtained in material of the Invar-type made in accordance with the present invention are given in Table IV. Proportional limits of 60,000 to 70,000 pounds per square inch are readily developed in comparison with about 20,000 pounds per square inch for ordinary Invar-type alloys.

40

Table IV

| Property                                    | Softened condition | Aged condition                               |
|---------------------------------------------|--------------------|----------------------------------------------|
| Tensile strength... p. s. i.                | 76,000 to 88,000   | 136,000 to 180,000                           |
| Yield strength... p. s. i.                  | 40,000 to 48,000   | 97,000 to 144,000                            |
| Proportional limit... p. s. i.              | 20,000 to 32,000   | 52,000 to 75,000                             |
| Brinell hardness... 130 to 160              | 130 to 160         | 225 to 425                                   |
| Reduction in area... percent                | 72 to 80           | 36 to 18                                     |
| Elongation... do                            | 39 to 43           | 17 to 11                                     |
| Minimum coefficient of expansion... per °F. |                    | $1.2 \times 10^{-6}$ to $2.2 \times 10^{-6}$ |
| Inflection temperature... °F.               |                    | 500° to 250°                                 |

55

In order that those skilled in the art may have a better understanding of the present invention, illustrative examples are given in Table V of the composition and properties of age hardened alloys made in accordance with the present invention.

Table V

| Alloy No. | Nickel |           | Titanium |              | Carbon | Min. coef. expansion $\times 10^{-6}$ °F. | Brinell hardness | Inflection temp. |
|-----------|--------|-----------|----------|--------------|--------|-------------------------------------------|------------------|------------------|
|           | Actual | Effective | Actual   | Non-carbidic |        |                                           |                  |                  |
| 1.        | 39.5   | 36.1      | 1.56     | 1.44         | 0.03   | 1.3                                       | 290              | 480              |
| 2.        | 40.6   | 36.0      | 2.06     | 1.90         | 0.04   | 1.6                                       | 321              | 480              |
| 3.        | 40.2   | 34.8      | 2.36     | 2.24         | 0.03   | 1.6                                       | 350              | 430              |
| 4.        | 41.4   | 35.1      | 2.73     | 2.65         | 0.02   | 2.1                                       | 363              | 420              |
| 5.        | 41.1   | 34.5      | 2.80     | 2.72         | 0.02   | 2.0                                       | 366              | 390              |
| 6.        | 44.2   | 38.1      | 2.70     | 2.58         | 0.03   | 2.3                                       | 364              | 570              |
| 7.        | 47.1   | 41.1      | 2.60     | 2.52         | 0.02   | 3.4                                       | 338              | 650              |
| 8.        | 41.8   | 34.7      | 3.04     | 2.96         | 0.02   | 1.6                                       | 380              | 390              |
| 9.        | 47.1   | 41.1      | 2.58     | 2.50         | 0.02   | 3.4                                       | 338              | 650              |
| 10.       | 52.0   | 45.9      | 2.64     | 2.56         | 0.02   | 4.9                                       | 319              | 810              |

The present invention provides a method of producing improved age hardenable iron-nickel alloys, and articles of manufacture made therefrom, possessing predetermined high mechanical properties and expansion characteristics and containing as essential ingredients about 1% to about 5% titanium, about 34.4% to about 60% total nickel and the balance substantially iron, in which carbon may be present up to about 0.2%, which comprises incorporating in an iron-nickel alloy a selected titanium content within said range such that  $Ti - 4 \times C$  lies between about 1% and 4.25%, the selected titanium content corresponding to the predetermined desired mechanical properties, for example, the desired hardness, and being larger the higher said desired properties; the nickel content of said alloy being proportioned within said range in accordance with the following formula:

$$\text{Total Ni} = \text{Effective Ni} + K(Ti - 4 \times C)$$

where the effective nickel is selected within the ranges of about 32% to about 50% to correspond to the predetermined desired low expansion characteristics,  $K$  being a constant having a value of about 2.4, and Ni, Ti and C being respectively the weight percentage of nickel, titanium and carbon, whereby an improved age hardenable iron-nickel alloy is obtained combining low expansion properties with high mechanical properties, including high hardnesses, in the age hardened condition.

The present invention contemplates improved age hardenable and age hardened articles of manufacture made of the alloys of predetermined low expansion characteristics provided by the present invention. Typical illustrative examples of uses for cast and wrought alloys of this type where strength, high proportional limit hardness or wear resistance are required combined with predetermined low expansion characteristics include turbine shafts; colloid mills; looms; dividing heads and accurate gear work; dies; reamers; boring bars; gauges; machine parts including glass machines; lead screws; valves; Diesel injector pumps and valves; thermostats; rolls; rolling mill frames and screw down; platinum, tantalum and glass lined autoclaves and clad materials; diamond and carbide tipped tool shanks including drills; proportioning pumps and meters; and for highly polished articles, such as reflectors, where the ease of polishing of a hard material is important, as is the absence of warping in subsequent use.

I am aware of the invention described in U. S. patents to Pilling and Merica, including U. S. Patent No. 2,048,163, and I do not claim any of the subject matter disclosed therein. The present invention is an improvement in the art of low expansion iron-nickel alloys.

Although the present invention has been described in conjunction with preferred embodiments, it is understood that modifications and variations may be resorted to without departing from the spirit and scope of the invention, as those skilled in the art will readily understand.

I claim:

1. As an article of manufacture, an age hardened iron-nickel-titanium alloy having minimum coefficient of expansion and containing in weight percentage 39.3% to 44.3% nickel; 2% to 3.5% titanium; 0.001% to 0.07% carbon; the percentage of titanium and carbon being such that

$$15 \quad Ti - 4 \times C$$

lies between 2% and 3.25%, and the percentage of nickel, titanium and carbon being such that

$$20 \quad \text{Total Ni} - K(Ti - 4 \times C)$$

lies between 34.5% and 36.5%,  $K$  being a constant having a value of about 2.4 and Ni, Ti and C being respectively nickel, titanium and carbon in weight percentage; and the balance being substantially all iron whereby a novel age hardened iron-nickel-titanium alloy is obtained having a unique combination of properties, including minimum coefficient of expansion and inflection temperatures above approximately 250° F. together with high hardness exceeding about 225 Brinell.

2. The article of manufacture set forth in claim 1 constituted of the alloy which has been subjected to cold work.

3. As an article of manufacture, an age hardened iron-nickel-titanium alloy having minimum coefficient of expansion and containing in weight percentage 39.3% to 44.3% nickel; 2% to 3.5% titanium; 0.001% to 0.2% carbon; the percentage of titanium and carbon being such that

$$40 \quad Ti - 4 \times C$$

lies between 2% and 3.25%, and the percentage of nickel, titanium and carbon being such that

$$45 \quad \text{Total Ni} - K(Ti - 4 \times C)$$

lies between 34.5% and 36.5%,  $K$  being a constant having a value of about 2.4 and Ni, Ti and C being respectively nickel, titanium and carbon in weight percentage; and the balance being substantially all iron whereby a novel age hardened iron-nickel-titanium alloy is obtained having in the aged condition a unique combination of properties, including minimum coefficient of expansion and inflection temperatures above approximately 250° F. together with high hardness exceeding about 225 Brinell.

ALBERT M. TALBOT.